

March 26, 1957

R. GABLER

2,786,732

PROCESS FOR RAISING THE MELTING POINT OF POLY-E-CAPROLACTAM  
FILAMENTS, THREADS AND YARNS BY TREATMENT WITH GASEOUS  
FORMALDEHYDE AND PRODUCTS PRODUCED THEREBY

Filed March 3, 1953



INVENTOR.  
RUDOLF GABLER  
BY *Arnold S. Martin*  
ATTORNEY

## 1

2,786,732

**PROCESS FOR RAISING THE MELTING POINT OF POLY- $\epsilon$ -CAPROLACTAM FILAMENTS, THREADS, AND YARNS BY TREATMENT WITH GASEOUS FORMALDEHYDE AND PRODUCTS PRODUCED THEREBY**

Rudolf Gabler, Tamins, Switzerland, assignor to *Inventa A. G. fuer Forschung und Patentverwertung, Zurich, Switzerland*

Application March 3, 1953, Serial No. 340,051

Claims priority, application Switzerland August 20, 1949

6 Claims. (Cl. 8—115.5)

This invention relates to the production of products with high melting points from polyamides. More particularly, the invention relates to a process for improving the properties of shaped articles prepared from  $\epsilon$ -caprolactam. Among these shaped articles are threads and yarns for general use, and cord as well as cord fabrics for tires. This application is a continuation-in-part to the co-pending applications Ser. Nos. 176,052 and 176,053 both filed July 26, 1950, now abandoned.

The improvement in the properties of the above mentioned articles is brought about, generally speaking, by a subsequent treatment of the polyamides with aldehydes.

Attempts have already been made to improve the properties of fibers, threads and other articles made therefrom, which were derived from synthetic linear polyamides, by subsequent treatment of the same with formaldehyde. Treatments of this kind have been carried out either by dissolving the polyamide and heating it with formaldehyde; or by treating the shaped polyamide with formaldehyde in a soaking liquid, such as water or alcohol in the presence of an acid catalyst. By this treatment, the formaldehyde is attached to the nitrogen atoms or polyamide chains in the form of methylol groups. The methylol polyamides obtained by evaporation of the solvent or soaking means are easily soluble products having, as a rule, lower melting points than the starting material.

It has also been discovered that, by heating the methylol compounds, interlocked insoluble products may result, whose melting point is considerably above that of the starting material. It may be assumed that in these interlocked polyamides the neighboring molecular chains are connected by  $\text{CH}_2$  bridges.

These products are, however, not satisfactory in the further processing. If the polyamides undergo formaldehyding treatment in solution, the resulting products cannot be spun readily. Even when formaldehyding is carried out in the presence of soaking means, the structure of the polyamides is so extensively altered that while the treated product is distinguished by a high melting point and improved elasticity, it has completely lost its other typical polyamide characteristics, in particular the high tensile strength.

This is also true of another known method which consists in heating undrawn filaments and other articles derived from nylon with an alcohol and with formaldehyde vapors in the presence of an acidic catalyst. While this process is aimed at and actually yields articles of high elasticity, it is not useful for the production of fibers, threads and the like exhibiting high tensile strength.

The reduction in strength is probably due to the loosening of the structure by the soaking means and, furthermore, the space required by the methylol groups formed in the first reaction step has a loosening effect and a 70 partial demolition of the polyamide chains finally seems to take place in the acid medium.

## 2

Certain disadvantageous properties of polyamide fabrics, which are hardly disturbing in other applications, as for example the always present plastic stretch, a certain thermoplasticity at temperatures such as occur in highly stressed tires, as well as their low affinity for rubber or rubber-like coverings hitherto still stood in the way of general use of polyamide cord fabrics.

There has been no lack of attempts to eliminate these disadvantages and patent literature contains a series of 10 processes suitable for removing one or the other of the deficiencies mentioned.

Thus, for instance, it was possible to improve the affinity for rubber of the linear polyamide, such as nylon, by treating it with diisocyanates. This treatment, however, did not effect an improvement with respect to 15 plastic stretch and the thermoplastic range. Other treatments were likewise not fully successful.

The inventor has discovered that the above-mentioned 20 disadvantages of the formaldehyding and other treatments used hitherto can be completely avoided if the products undergoing the treatment are first subjected to a cold-drawing operation and thereafter treated with gaseous formaldehyde in the absence of all means adapted to dissolve or soak the treated material. Since the formation of methylol bridges takes place with simultaneous removal of water, this reaction is accelerated when working in the absence of water. Obviously, the acceleration is so effective that the intermediary alkylol stage is of short duration and the formation of methylol bridges 25 is achieved under essential maintenance of the original crystalline structure.

As a rule, the materials to be treated are only subjected 30 to a cold-drawing process, i. e. a drawing process occurring at room temperature, in a single stage. In some 35 cases, for instance for cord yarns, it is advantageous to operate in two stages, carrying out a hot-drawing operation subsequently to the cold-drawing.

The cold-drawing operation brings about an increase 40 in the length of the fibers by about 250—400%; hot-drawing at temperatures of about 180° C. effects a further increase in length of 20—50%.

The drawing operation may be carried out in any 45 known manner. The yarns may, e. g. be wound onto perforated metal cylinders, while being drawn. If a twisting operation is to be combined with the drawing operation, i. e. if thread formation is intended, the fibers are rewound from bobbins onto perforated metal cylinders, the tensioning force on the thread being at least 1 gram/den.

50 On the perforated metal cylinders, the threads are wound with a large angle of crossing, e. g. an angle of 30—45°. This is done for the purpose of making the inner layers of thread easily accessible to the agents with which they are subsequently treated; the washing liquids 55 during the cleansing stage, dry air during the drying step, and vapors of aldehyde during the aldehyde operation. The three operations could also be carried out subsequently in the same apparatus (see drawing).

The temperature range for the subsequent formaldehyding with gaseous formaldehyde lies between 120° and 60 180° C., preferably at 140° C. I may proceed by letting the formaldehyde vapors, which are developed from paraformaldehyde or some other material furnishing formaldehyde, react with the polyamide by means of a heated 65 inert gas, for example nitrogen. The reaction may be considerably accelerated by the use of pressure, but may also be carried out at atmospheric pressure.

After such treatment, these threads are outwardly unchanged, but their melting point has been raised to 330° C. The raising of the melting point is dependent on the degree of formaldehyding. In general, the melting point of the formaldehyded polyamide is 80—150° C. above the

original melting point, corresponding to a weight increase of 8 to 14%.

The filaments from synthetic linear polyamides are outwardly unchanged after the formaldehyding. The mechanical testing shows a practically unchanged strength, but reduced total extension and increase of the elastic portion of the latter. This is of great importance in the manufacture of cord for tires.

The total extension of a polyamide fiber, as is well known, is composed of a plastic and an elastic part. In the case of normal textiles the mechanical strains on the material generally lie within the elastic limit of the extension, so that permanent deformations are hardly to be feared. On the other hand, the cord fabric lining of airplane tires, for instance, must withstand tremendous strains of stretching at the moment of landing, whereby the limit of elasticity is exceeded and permanent deformations occur. This can reach a point at which the landing gear, after repeated landings and as a result of change in the shape of the tires, can no longer be retracted into the apertures provided in the body of the plane. Similar changes in shape may occur when vehicle tires are under constant strain and are strongly heated by friction with the ground. The mechanical tests of synthetic linear polyamides subjected to subsequent treatment with aldehydes indicate with increasing addition of interlocking molecular groups not only a reduction of total extension, but also a recession of the proportion of plastic extension. Beginning with a certain degree of interlocking, the plastic deformation becomes zero and the material consequently exhibits only elastic deformation.

For every possible combination of a polyamide fiber and an aldehyde used for subsequent treatment, there is an optimum as regards proportional absorption of interlocking groups which in general lies between 8% and 15%. When this optimum is exceeded, the tensile strength of the treated fibers decreases rapidly, so that finally the value as a textile is completely lost. The extension exhibits, above the interlocking optimum, a strong increase. At the same time, the extension becomes completely elastic and the material acquires rubber-like characteristics.

As a result of the process according to the invention, the strength of adhesion of the polyamide fiber to rubber or rubber-like natural and synthetic materials is improved. The effect of the formaldehydization and/or treatment with other aldehydes may be conceived of as blocking the anti-rubber acid-amide groups whereby the hydrocarbon character of the molecular chains becomes more pronounced. The strength of adhesion of various polyamide materials to rubber was tested with suitable measuring apparatus which consisted in principle in vulcanizing a cord thread of given titer and twist, into a rubber cube and extracting it by means of attached weights. Designating the adhesive strength of an untreated polyamide yarn as 100, the adhesive strength of polyamide yarns treated with aldehydes was found to be between 146 and 182, depending on the degree of aldehyding.

Another important improvement brought about by the aldehyde treatment is a decrease of the polyamides in their heat sensitivity. This is important for ordinary fabrics undergoing ironing, as well as for cord fabrics which become heated due to friction.

As regards the aldehydes to be used in the treatment according to the invention, it has been found that not only formaldehyde, but also higher saturated aliphatic aldehydes may be successfully used. They may be monovalent or polyvalent. As examples I mention acetaldehyde, propionaldehyde and glyoxal. The carrying out of the process according to the invention is done in the same manner regardless of the aldehyde used.

The accompanying drawing shows diagrammatically and by way of example a system adapted for carrying out the process according to the invention.

The system comprises a pressure vessel 1 provided with manometer 2 and high pressure valve 3. A perforated spool 4 to carry the material to be treated is provided inside the pressure vessel. In order to circulate the heated treatment vapors through the pressure vessel, means are provided comprising a container 5, a tube system 6, a cooler 7, a compressor 8 and a pre-heater 9.

By the "absence of all means adapted to dissolve or soak the treated material" it is intended to exclude the presence of solvents as well as swelling agents. Water and alcohols are the most common swelling agents; phenol is a solvent if used per se, a swelling agent in aqueous solution. All these, as well as similarly acting substances, should be absent.

As mentioned before, the known aldehyding processes operate by allowing the polymers to swell in the presence of acid agents and/or water, alcohols, phenols, and so on. This causes a considerable decrease in the strength of the textiles.

The invention will now be described in the following examples, but it should be understood that these are given by way of illustration and not of limitation, and that many modifications in the details may be made without departing from the spirit of the invention.

#### Example 1

A polymerization product consisting of poly  $\epsilon$ -caprolactam with an intrinsic viscosity of 2.4 was spun from the melt at 285° C. into a yarn consisting of 80 filaments and having a total titer of 1325 denier. After pre-twisting to 110 trs. p. m., the yarn was cold-drawn at the ratio of 1:1.50. The yarn, which now had a total titer of 265 at 20-25 trs. p. m. and a tensile strength of 6.0 g./den., was wound onto a metal cylinder of 150 millimeters diameter and 180 millimeters length, while being subjected to a tensile force of 3 g./den.

The yarn was then washed under pressure in a conventional washing device, in order to eliminate monomer components and remainders of spinning preparations, and was thereafter thoroughly dried to a water content of less than 0.2%. Three bobbins of the yarn thus obtained were formaldehyded in an apparatus as described and illustrated, for four hours at a temperature of 160° C. and 5-6 p. s. i. with a nitrogen stream laden with formaldehyde vapors.

After the termination of the treatment, the weight of the yarn had increased by 13.5% and the melting point had gone up from 214° C. to 330° C. The tensile strength of the yarn was 5.8 gram/denier.

#### Example 2

A yarn of poly- $\epsilon$ -caprolactam with a total titer of 265 denier (80 filaments) and 20-25 trs. p. m., as obtained in the cold-drawing process described in Example 1, was again subjected to a drawing operation at 180° C. to about 125% of its original length. The yarn then exhibited a tensile strength of 5.8 g./den. and 12.6% extension, of which 85% were elastic extension. In the combined heat-drawing and twisting process, the twist of the yarn was increased from 20-25 trs. p. m. to 130-150 trs. p. m. From the bobbins, on which it was drawn, the yarn was rewound onto perforated metal cylinders with each single thread being subjected to a tensile force of 1 g./den. After having been washed and dried in a conventional manner, the material on the cylinders was treated in the described apparatus in a nitrogen atmosphere with formaldehyde vapors at 140-145° C. and 6-7 p. s. i., until the increase in weight amounted to 12.5%. From the formaldehyded yarn a cord thread 220 den. 2 S twist 5 Z twist was made having a final titer of 2195 den.

Tests made with the material showed its tensile strength to be 5.1 gram/den., and the total elastic extension of 8.7%. The melting point had gone up from 214° C. to 270° C.

What I claim is:

1. The process for raising the melting point of articles consisting of poly- $\epsilon$ -caprolactam synthetic linear polyamide fibers, which comprises cold-drawing said fibers to about 350%–400% of their original length, drying the same to free them completely from water, and thereafter reacting them with dry gaseous formaldehyde, at a temperature ranging from 120 to 180° C. in an environment substantially consisting of an inert gas, and being free from catalysts, for a period of several hours, until the weight of the treated material has increased by about 8–14%.

2. The process as set forth in claim 1, wherein the reaction of the articles with the gaseous formaldehyde is performed in a stream of nitrogen.

3. Poly- $\epsilon$ -caprolactam synthetic linear polyamide filaments, threads, and yarns, produced by subjecting said filaments, threads and yarns to a cold-drawing process, whereby they are extended to from 350%–400% of their original length, then drying the same to free them completely from water, and thereafter reacting them with dry gaseous formaldehyde, at a temperature ranging from 120 to 180° C. in an environment free from catalysts and substantially consisting of an inert gas for a period of several hours, said treated material having a weight increase, as compared to the starting material, of from 8–14%, and a melting point raised by from 80 to 150° C.

4. A cord fabric for vehicle and airplane tires made of poly- $\epsilon$ -caprolactam synthetic linear polyamide fibers produced by subjecting said polyamides to a cold-drawing process whereby they are extended to 350%–400% of their original length, dried, and thereafter reacted with dry gaseous formaldehyde, at a temperature ranging from 120 to 180° C. in an environment free from catalysts and substantially consisting of an inert gas for a period of several hours and having as a result of said reaction a weight increase, as compared to the starting material, of about 8–14% and a melting point increased by 80–150° C.

5. The process of improving poly- $\epsilon$ -caprolactam

synthetic linear polyamide fibers to be made into cord fabric, which comprises cold-drawing said fibers to from 350% to 400% of their original length, drying the same to free them completely from water, and thereafter reacting them with dry gaseous formaldehyde, at a temperature ranging from 120 to 180° C. in an environment free from catalysts and substantially consisting of an inert gas for a period of several hours until the weight of the treated material has increased by about 8–15%.

10 6. The process of improving poly- $\epsilon$ -caprolactam synthetic linear polyamide fibers to be made into cord fabric, which comprises subjecting said fibers to a cold-drawing operation at room temperature until an extension of the fiber length of about 250–400% has been reached, then subjecting the fibers to a hot-drawing operation at a temperature of about 170–190° C. until a further extension of the fibers of about 20 to 50% is obtained, drying the same to free them completely from water, and thereafter reacting them with dry gaseous formaldehyde, at a temperature ranging from 120 to 180° C. in an environment free from catalysts and substantially consisting of an inert gas for a period of several hours until the weight of the treated material has increased by about 8–15%.

15 25 20 25 References Cited in the file of this patent

UNITED STATES PATENTS

|           |               |       |               |
|-----------|---------------|-------|---------------|
| 2,430,953 | Schneider     | ----- | Nov. 18, 1947 |
| 2,434,247 | Lewis et al.  | ----- | Jan. 13, 1948 |
| 2,516,562 | Graham        | ----- | July 25, 1950 |
| 2,540,726 | Graham et al. | ----- | Feb. 6, 1951  |

FOREIGN PATENTS

|         |               |       |               |
|---------|---------------|-------|---------------|
| 582,520 | Great Britain | ----- | Nov. 19, 1946 |
|---------|---------------|-------|---------------|

OTHER REFERENCES

Hall: Silk Journal and Rayon World, April 1947, pages 30–32.